

1

2,727,826

IMAGE TRANSFER MATERIAL AND METHOD  
OF MAKING IT

Harold G. Greig, Princeton, N. J., assignor to Radio Corporation of America, a corporation of Delaware

No Drawing. Application September 30, 1950,  
Serial No. 187,827

5 Claims. (Cl. 106—289)

The present invention relates to improvements in a process of electrostatic printing and to improved materials for use in such a process.

One well known process of electrostatic printing comprises the following steps: (1) inducing an electrostatic charge on a surface of a plate coated with a film of a photoconductive insulating material, (2) exposing the charged plate to a light image for the purpose of releasing the charge at every point exposed to the light, (3) contacting the plate with a particulate coloring material, usually in the form of colored particles adhering to the surfaces of small glass beads, wherein the colored particles are detached from the beads and adhere to the plate at every point where the charge has not been released by the light, and (4) contacting the colored image with a sheet of paper or the like to transfer a copy of the image to the paper.

In the above type of process, many types of colored materials have been tried for developing the latent image. Among these coloring materials have been: metal bronzing powders, colored gums, hard waxes, and resins, dyed resins, dyed lycopodium powder, powdered sulfur, or talcum powder, where the powders are dyed substantially throughout, also powdered dyes, and carbon dust.

Although all of these may be used with some degree of success, they possess certain disadvantages. Most of them do not provide adequate depth of color and some have a melting point higher than the scorching temperature of paper so that it is difficult to fix the transfer print by heating it.

The present invention is directed particularly to an improved type of medium for applying color to any latent image formed on an electrostatically charged plate where the image area is charged either negatively or neutral and the remainder of the plate is charged positively. The preferred form of improved coloring medium, according to the present invention, does not have the disadvantages pointed out in connection with previously used media.

In general, the improved coloring medium of this invention comprises a substantially spirit-insoluble powder having good dielectric properties and having each particle of the powder coated with a precipitated dye. The powder particles are not dyed throughout; neither is the dye merely smeared on the particle surface; instead, the dye is precipitated on the surface.

One object of the present invention is to provide an improved medium for imparting transferable color to any latent image when the latent image is charged negatively and the area surrounding it is charged positively.

Another object of the invention is to provide an improved process for imparting color to a latent image comprising an uncharged area surrounded by an area which is electrostatically charged positively.

Another object of the invention is to provide an improved medium for developing a latent image carrying a negative electrostatic charge.

Another object of the invention is to provide an improved developer powder for electrostatically charged

2

latent images, which produces an excellent blue-black color relatively insensitive to heat, acid, alkali, and the common solvents such as water, alcohols, and the hydrocarbons.

Still another object of the invention is to provide an improved developer powder for use in facsimile systems. These and other objects will be more apparent and the invention will be more readily understood from the detail description of the invention which follows.

10 The improved coloring matter of the present invention is prepared by taking a finely powdered material having good dielectric properties as a base and precipitating a dye onto the surface of the powder. The precipitated dye is preferably a reaction product of two spirit-soluble dyes which may be mixed to produce a spirit-insoluble product. The powder base is preferably one which has a relatively low melting point but, less desirably, may be a material of high melting point. By "spirit-soluble" is meant soluble in any of the lower alcohols or as this term is commonly used in the dyeing industry. By "good dielectric properties" is meant the ability to hold an electrostatic charge for at least about 10 seconds without appreciable leakage.

## Example

25 An example of preparation of a preferred embodiment of the material according to the invention is as follows: 40 parts by weight of sulfur in finely divided form, as, for example, sublimed sulfur flowers, is formed into a thin slurry or paste by mixing with 50 parts by weight of methanol. 1.5 parts by weight of spirit-soluble nigrosine dye SSB, Color Index No. 864, is added to the paste and the mixture is stirred until the dye is completely dissolved in the alcohol and all of the sulfur is thoroughly dispersed. To this is then added 1 part by weight of a spirit soluble dye that is the condensation product of the dye:



30 and an organic base to give solvent solubility, such as tri-  
35 amylamine, or an equivalent amount of any other of several well known dyes which will react with the nigrosine to precipitate a black dye. Other suitable dyes are the spirit-soluble fast black dyes which can be prepared as described in United States Patent 2,095,077. For example, one may use the spirit soluble fast black dye made from the dye:



50 which is condensed with an organic base to give solvent solubility according to the process described in U. S. Patent 2,095,077.

55 60 Enough of the second dye is added, in any case, to cause complete precipitation of the nigrosine. The two colors are individually soluble in alcoholic spirits, but when a solution of one is added to a solution of the other, an insoluble black pigment is formed. When they are mixed in the presence of sulfur, as described, the pigment is precipitated onto the sulfur particles.

65 The product is isolated by filtering. Traces of excess color can be removed by washing the filter cake with a small amount of methanol or with warm water until the filtrate runs clear of color.

70 75 The product is then dried at a temperature below the melting point of sulfur. It dries to a finely divided black

powder. In this form, the powder can be used, under some conditions, as an electrostatic dusting powder, but, for most purposes, its action can be greatly improved by grinding it in a ball mill. Conditions and time of ball milling are important from the standpoint of obtaining optimum electrostatic properties in the product. If it is desired to utilize the powder as a negative developer, i. e., one which will adhere to the exposed areas of a positively charged plate, one hour of ball milling is suitable for the size sample used in the example. For larger samples, ball milling should be longer. Times of up to 4 hours have been used. If the powder is not ground, the image produced is faint and blurred and may have a dirty background. The pure pigment alone, without the sulfur base, gives similar results. As ball milling proceeds, the powder, when tested, will be found to adhere more strongly to the image areas and to be repelled better by the charged background of the plate. If ball milling is continued for too long a time, the powder begins to adhere very strongly to the image areas, when tested, making transfer to a sheet of paper, and the cleaning of the plate, more difficult. There is also a tendency for the powder to lose color strength since the pigment coat is slowly removed as ball milling continues, with the color adhering to the sides of the mill. Time and conditions of grinding depend upon amount and form of color pigment deposited and size and form of the base particles.

#### Printing procedure

One form of printing procedure that has proved successful with the above described developer powder is the following. A polished aluminum plate is provided with a surface coating of red, amorphous selenium. This plate is charged in the dark by passing it under a positive corona discharge at high potential; i. e., 6 to 8 kv. on 5 0.003" diameter wires placed  $\frac{1}{16}$ " above the plate. The charged plate is exposed to a light image by any well known technique, such as contact printing, projection, or kinescope scanning, and the latent image is developed; that is, transferable color is imparted to it, by flowing a mixture of the developer powder and glass carrier beads over the exposed surface. The powder adheres to the selenium, probably by triboelectric effect, in the areas where the induced charge has been released by the exposure to light. It is repelled by the unexposed areas 45 which still retain the induced charge. Thus, a negative of the image is produced.

Transfer of a copy of the image negative to a sheet of paper, or the like, is made by placing the sheet on the plate and passing it under the corona wires with 50 the polarity reversed. The paper is thus given a negative electrostatic charge. The image taken off on the paper in this manner is then fixed by heating to the fusing temperature of the powder.

Glass beads of various sizes can be used to carry the powder. Beads ranging in diameter from 0.015" to 0.040" have given good results. An amount of powder which is about 1 to 2% of the weight of the beads has been found to give optimum results. This varies slightly with bead size and type of glass.

Images can be developed on insulating surfaces other than photoconductive insulators such as selenium. Varnished or resin coated metal plates or glass plates can, for example, be used in a process which differs from that described above in that after a corona-induced positive charge has been applied to the surface, this charge is removed locally to form a latent image by contact with a conductor. The developer powder is then applied to the plate and is retained in the image areas. The improved developer powder can thus be used to apply color to any latent image having an electrostatic charge contrasting with that of the surrounding area, when the image area, itself, either carries no charge or is negatively charged. The image should not absorb the dye or the powder to any extent. Usually, the

color adheres most strongly to the edges of the image at the boundary between the areas of contrasting charge. The color can be made to appear over the whole image surface, however.

In preparing the improved developer, concentrated solutions of the dyes should be used to give best results. This is probably because precipitation of a pigment from a concentrated solution normally favors formation of larger pigment particles. Either dye can be added to the sulfur slurry first and precipitated by addition of the other color dry or in solution.

Although it is preferred to use a base particle, such as sulfur, having a relatively low melting point compared with the scorching temperature of paper, many other materials can be used in finely divided form with somewhat poorer results. Examples are lycopodium powder, diatomaceous earth, glutamic acid, and 1-phenyl-3-methyl-5-pyrazolone. It is necessary only that the particle have good dielectric properties and that it be substantially insoluble in the alcohols used to dissolve the dyes. Where the particle has too high a melting point to be set by fusing on the paper, setting may be accomplished by spraying with lacquer or some other binder.

Any combination of spirit-soluble dyes may be used which will react to precipitate a color pigment. Nigrosine is preferred as one of the two but any one of many known spirit-soluble dyes can be mixed with it or they can be mixed together with no nigrosine present. Others are Solventol Blue, Solventol Blue 6G, and Solventol Black Z-3164.

The preferred form of the developer powder which has been described has proved to have exceptionally fine properties for making negative electrostatic prints in one type of facsimile system. The powder produces black prints of good contrast. It is easy to prepare, requiring little or no classification in order to obtain a narrow range of particle size. It is clean to handle and may be removed relatively easy from hands and clothing without staining. It is not tacky and has no tendency to wet a selenium surface. Thus, it can be cleaned readily from the printing plate, a factor of importance in a continuous printing process. The pigments also have excellent light fastness. There has thus been described an improved developer powder for latent images carrying either a negative electrostatic charge or no electrostatic charge when the surrounding areas are positively charged, and an improved process for applying transferable color to an electrostatically charged latent image. The same effect cannot be obtained by merely grinding together base particles and pigment or dye particles. For example, 20 parts sulfur and 4 parts carmine were ball milled. This gave a reverse print using the process described above. That is, the color adhered to all positively charged areas.

I claim as my invention:

1. An image transfer material comprising a substantially spirit-insoluble, inert, dielectric powder having a surface coating of a spirit-insoluble, precipitated organic pigment, said pigment having been prepared by precipitating spirit-soluble nigrosine with a spirit-soluble dye selected from the class consisting of the condensation product of the dye



and an organic base to give solvent solubility and the condensation product of the dye



5

and an organic base to give solvent solubility upon said powder while said powder is suspended in a spirit medium.

2. A material according to claim 1 in which said powder is sulfur.

3. A material according to claim 1 in which said surface coating is a precipitant which is the reaction product of spirit-soluble nigrosine and a spirit-soluble black dye which is the condensation product of the dye



and an organic base to give solvent solubility.

4. A method of making an image transfer material comprising suspending a substantially spirit-insoluble inert dielectric powder in a spirit medium and then precipitating spirit-soluble nigrosine with a spirit-soluble dye selected from the class consisting of the condensation product of the dye



6

and an organic base to give solvent solubility and the condensation product of the dye



and an organic base to give solvent solubility on the surface of said powder while suspended in said spirit medium.

5. A method according to claim 4 in which said powder is sulfur.

**References Cited in the file of this patent**

| UNITED STATES PATENTS |           |                              |
|-----------------------|-----------|------------------------------|
| 15                    | 2,095,077 | Payne ----- Oct. 5, 1937     |
|                       | 2,118,512 | Hucks ----- May 24, 1938     |
|                       | 2,221,776 | Carlson ----- Nov. 19, 1940  |
|                       | 2,297,691 | Carlson ----- Oct. 6, 1942   |
| 20                    | 2,357,809 | Carlson ----- Sept. 12, 1944 |
|                       | 2,502,254 | Glassman ----- Mar. 28, 1950 |

25